

M. A. ADAM, J. STEVENSON AND A. T. MABBITT,

DETINNING OF TINNED IRON SCRAP,

APPLICATION FILED AUG. 31, 1920

1,379,237.

Patented May 24, 1921.



Fig.1



Fig.2.

INVENTORS

M. A. Adam

J. Stevenson

A. T. Mabbitt

*H. R. Kerstake*, ATTORNEY

# UNITED STATES PATENT OFFICE.

MATTHEW ATKINSON ADAM, JOHN STEVENSON, AND ALAN THOMAS MABBITT, OF LONDON, ENGLAND; SAID STEVENSON AND SAID MABBITT ASSIGNORS TO SAID ADAM.

## DETINNING OF TINNED IRON-SCRAP.

1,379,237.

Specification of Letters Patent. Patented May 24, 1921.

Application filed August 31, 1920. Serial No. 407,250.

To all whom it may concern:

Be it known that we, MATTHEW ATKINSON ADAM, residing at 57, Lincoln's Inn Fields, London, W. C. 2, England, JOHN STEVENSON, 5 residing at 28 Talbot road, Bayswater, London, W. 2, England, and ALAN THOMAS MABBITT, residing at 3 Wallwood road, London, E. 11, England, all subjects of the King of Great Britain and Ireland, have invented 10 certain new and useful Improvements Relating to the Detinning of Tinned Iron-Scrap, of which the following is a specification.

This invention relates to the recovery of 15 tin in the wet way from tinned iron, *e. g.*, tin plate scrap.

It has hitherto been proposed to use strong boiling solutions of ferric chlorid to dissolve tin from tinned iron scrap, and then after 20 adding phenol and sulfuric acid to the drawn off solution, to electrolyze the same. A lead cathode and a cloth covered anode were proposed, and the separated tin was proposed to be collected at the bottom of the 25 electrolyte. (See Ramos Garcia, British Patent No. 18726 of 1890.)

In this process as described, filtering of the solution was employed, and regeneration of the dissolving fluid effected by the 30 addition of ferric chlorid crystals intermittently collected and utilized after volatilization. Also, owing to the additions used for electrolysis, the solution could not be employed over again without treatment.

More recently weak solutions of ferric chlorid and hydrochloric acid have been tried on an industrial scale to recover tin from tinned iron scrap by dissolving tin and afterward depositing tin from the solution 40 by electrolysis in separate cells with stationary cathodes; the solution being circulated very slowly through the electrolytic cells. Considerable difficulties have arisen in the industrial utilization of this type of 45 process, *inter alia*, owing to the slow rate of solution of the tin, and to the fact that the yield of tin in the electrolysis of the solutions does not approach in practice even the equivalent corresponding to stannic chlorid.

The object of the present invention is to 50 provide an improved process according to which both a rapid rate of solution and a rapid rate of recovery of tin may be effected

so that a continuous process on a commercial scale is provided.

The invention consists, in brief, in employing strong solutions of the chlorids of tin and iron, with or without a small percentage of added hydrochloric acid for dissolving the tin from the tinned iron scrap, 60 and circulating the solution through one or more electrolytic cells operating at high current densities from which the deposit is automatically removed, and preferably removing by electrolysis only about the same amount 65 of tin as has been dissolved in the scrap treatment.

In carrying the invention into effect in one form by way of example, we make a solution in water of ferric chlorid to a strength 70 of about 25%, adding about 1% hydrochloric acid. We then introduce metallic tin and permit this to be dissolved as far as practicable, *viz.*, until the solution contains:—

About 6½% stannous chlorid, and  
About 1½% stannic chlorid.

The ferric chlorid often contains some free hydrochloric acid, so the amount of hydrochloric acid added varies to a certain extent, but we prefer only to add such an amount that the total free acid in the mixture is not greater than say 3%. The solution resulting from the above mixture (which consists substantially of ferrous, 85 stannous and stannic chlorids and hydrochloric acid) is employed for removing the tin from the tin scrap, and we find it dissolved tin well at ordinary atmospheric temperatures from such scrap, and attacks iron 90 but little.

After solution of the tin, the liquor is electrolyzed as explained below, and the effluent from the cell subsequently employed for dissolving more tin. We prefer only to remove 95 a small proportion of tin in one passage through the electrolyzer, so that the composition of the dissolving liquor is not appreciably altered.

When ferric chlorid is saturated with tin 100 (it being reduced to ferrous chlorid in the reaction,) then tin and iron are in equilibrium in solution, and the resulting solution has no solvent action on tin. As the tin content is decreased, so the rate of activity of 105 the liquor as a solvent for tin increases

- rapidly, then the solution is sufficiently active for practical work for dissolving the tin from the tin plate when it contains say about 8% of tin chlorids as indicated above, 5 part being in the stannous and part in the stannic form (although as regards the tin salts, only the stannic chlorid is available for the solution of tin, it being converted to stannous chlorid by the reaction). The 10 liquor made as above described may be regarded as saturated with tin from the aspect of the solvent in question, that is to say, if a 25% ferric chlorid solution be allowed to take up as much metallic tin as is practicable, that is, until the resulting liquor 15 contains tin chlorids to approximately the extent described above, the liquor can be used to dissolve tin from tin plate by the action of the stannic chlorid content.
- 20 It is desirable from the electrolytic point of view to keep the tin content of the solution as high as possible (so that the ratio of stannous to stannic tin is high) but from the point of view of dissolving tin from 25 tin scrap it is desirable to keep some way from the saturation point in order to secure sufficiently rapid working.
- In the electrolysis we prefer so to choose the rate of (a) relative movement between 30 the cathode surface and the electrolyte, *e. g.*, the speed of rotation of the cathode, (b) liquid flow, and (c) current density, that only a comparatively small amount of the total tin content is deposited from the solution 35 as explained above, and that it is deposited in a non-coherent form.
- We have found that good results are obtained with a current density of about 450 amperes per square foot in a cell in which 40 the cathode is rotated at a peripheral speed of about 10 inches per minute, the liquid flow being about 10 gallons per hour through a channel between anode and cathode of about  $\frac{1}{2}'' \times 6''$ , and in this case the 45 amount of tin deposited from the solution was about 0.2 lb. per hour. If it be desired to treat a different volume of liquid, this will determine the rate of liquid flow, and according to the quantity of metal it is required to deposit from the solution, so the 50 current will be determined. In this way the cathode area is fixed, and the current density must be so chosen that a deposit suitable for removal by a light scraping action 55 is obtained. The conditions may, however, be varied, *e. g.*, by depositing a larger proportion of tin from the solution. If the area of the cathode be fixed, then the rate of rotation should be such that a non-adherent deposit is obtained with the given 60 current density. The rate of liquid flow and the size of the cell may be selected on the basis of the above figures according to the different conditions which may exist in materials under consideration, that is, for ex-

ample, the different amount of liquid to be treated.

Referring to the accompanying diagrammatic drawings—

Figure 1 represents a convenient arrangement of tanks and system generally; and 70

Fig. 2 indicates a convenient construction of electrolytic cell.

In the arrangement illustrated, the scrap suspended in baskets say of metal openwork 75 coated with acid-resisting enamel, is immersed in the dissolving solution and agitated therein in any suitable way as indicated by way of example in Fig. 1. Conveniently, the baskets *a* are suspended in pairs on the ends of a lever *b* supported from a carriage *c* on a runway *d*. They thus balance one another, and are easily manipulated by hand or mechanically to secure an intimate contact of the scrap with the liquid. 80 The carriage *c* is provided with raising and lowering gear *e*, so that the baskets are raised after treatment in tanks *f*, *g* or *h*, moved along the runway to a pair of washing tanks *i*, in which they are immersed in 85 water, and again preferably to a limewater tank *j*, or to a copper-depositing tank in which a slight deposit of copper is made on 90 the scrap to protect it from subsequent oxidation.

The store tank *u* is connected through piping *v* to the electrolytic cell *k*, after which it passes through a heater *w* to pipe *x*, whence it may be distributed to any pair 95 of tanks *f*, *g* or *h* at will.

The electrolytic cell *k* we prefer to use is formed as a semi-circular trough in which is disposed a drum cathode of length about equal to that of the trough.

A form of construction of electrolytic 105 cell is illustrated diagrammatically in Fig. 2, in which the trough is formed by a graphite bar *l* hollowed out and provided with holes *m* along its bottom for exit of the electrolyte. The electrolyte passes into 110 the trough cell from both sides *n* of the supply chamber over the edges of the graphite trough *l* through the exit passages *m* into a sump *o* whence it flows through a 115 number of ways *p* to the outlet pipe *q*.

The graphite bar is preferably impregnated with paraffin wax to exclude the electrolyte from the pores thereof. Electrical connection may be made conveniently by copper rods *2* passing through the end of 120 the cell and entering the cathode bar, care being taken that no access to this connection is possible by the electrolyte.

The drum cathode *r* is mounted upon a spindle above the trough *l*, and thus may 125 be rotated during action of the cell with part of its surface immersed in the electrolyte, the latter being caused to flow at a steady rate through the system as determined by a cock *t* (Fig. 1). A scraper *3* is 130

arranged to collect the metallic tin from the surface of the drum.

In operation of the system one of the inlet cocks, say *y*, is opened and the cock *t* set to give the required rate of flow of the electrolyte. In the tanks *f*, when sufficiently full, the baskets *a* are lowered for detinning, and the cock *y* closed, and, say *z*, opened. Thus the flow of electrolyte is not disturbed, but merely now transferred to the tanks *g*. Similarly, when detinning is complete in tanks *f*, the appropriate outlet cock is opened, and the electrolyte returned to the store tank *u* by means say of a pump 1.

Having now described our invention, what we claim as new and desire to secure by Letters Patent is:—

1. A process for the detinning of tinned iron scrap which consists in dissolving the tin in strong solutions of the chlorids of tin and iron approaching saturation and circulating the solution through an electrolytic cell operating at high current density and practically continuously removing the non-coherent deposit.

2. A process for the detinning of tinned iron scrap which consists in dissolving the tin in strong solutions of the chlorids of tin and iron approaching saturation with a small percentage of added hydrochloric acid and circulating the solution through an electrolytic cell operating at high current density and practically continuously removing the non-coherent deposit.

3. A process for the detinning of tinner iron scrap which consists in dissolving the tin in strong solutions of the chlorids of tin and iron approaching saturation and circulating the solution through an electrolytic

cell operating at high current density and practically continuously removing the non-coherent deposit, the solution employed being substantially saturated with tin throughout the whole of the process.

4. A process for the detinning of tinned

iron scrap which consists in dissolving the tin in strong solutions of the chlorids of tin and iron approaching saturation and circulating the solution through an electrolytic cell operating at high current density and practically continuously removing the non-coherent deposit, the amount of tin removed by electrolysis being only about the same amount as has been dissolved in the scrap treatment.

5. A process for the recovery of tin from tin scrap in which the tin is dissolved by a strong solution of the chlorids of tin and iron and the resulting solution electrolyzed, and rate of (a) relative movement between the cathode surface and the electrolyte, *e. g.*, the speed of rotation of the cathode, (b) liquid flow, and (c) current density, being so adjusted that only a comparatively small amount of the total tin content is deposited from the solution, and that it is deposited in non-coherent form.

6. A process for the detinning of tinned iron scrap which consists in dissolving the tin in strong solutions of approximately 8% of the chlorids of tin and approximately 25% of chlorids of iron and circulating the solution through an electrolytic cell operating at high current density and practically continuously removing the non-coherent deposit.

7. A process for the detinning of tinned iron scrap which consists in dissolving the tin in strong solutions of the chlorids of tin and iron approaching saturation and circulating the solution through an electrolytic cell operating at high current density and practically continuously removing only the tin dissolved from the tinned iron.

In testimony whereof we have signed our names to this specification.

MATTHEW ATKINSON ADAM.

JOHN STEVENSON.

ALAN THOMAS MABBITT.